

W. C. JOHNSON.  
METHOD OF TREATING COTTON FIBERS AND PRODUCTS.  
APPLICATION FILED DEC. 15, 1919.

1,396,960.

Patented Nov. 15, 1921.



*Fig. 1.*



*Fig. 2.*

Witness  
*James E. Allen.*

Inventor:  
*William C. Johnson.*  
By *Ward & Ward*

Attorneys

# UNITED STATES PATENT OFFICE.

WILLIAM C. JOHNSON, OF MEMPHIS, TENNESSEE.

## METHOD OF TREATING COTTON FIBERS AND PRODUCTS.

1,396,960.

Specification of Letters Patent.

Patented Nov. 15, 1921.

Application filed December 15, 1919. Serial No. 344,867.

To all whom it may concern:

Be it known that I, WILLIAM C. JOHNSON, a citizen of the United States, and residing at Memphis, in the county of Shelby and State of Tennessee, have invented a new and useful Improvement in the Method of Treating Cotton Fibers and Products, of which the following specification is a full disclosure.

My invention relates to the art or method 10 of forming condensed blocks of absorbent cotton fibers and to the resultant product.

For the purposes of understanding the present invention it is not essential to show machinery suitable to operating the process 15 on a large commercial scale, inasmuch as the present invention concerns the essential treatment steps and product, irrespective of any special mechanical instrumentalities.

Cotton-seed hulls have long been treated 20 to separate the fiber from the hull particle, the bran constituting a valuable feed product. The fiber is relatively short and knotty, and so far has not been adopted as a desirable paper pulp.

25 It is also well known that when such fiber is treated with a solution of caustic soda to dissolve out certain cellular components that the resultant fiber is highly absorbent.

This invention is not limited to the origin 30 of the cotton fibers, but has to do with the treatment of cotton fibers, linters or the like, which are relatively short, knotty and harsh, and it is essential to my process and product, that such fibers be chemically treated to render 35 the fiber very absorbent, and then mechanically treated to straighten and unify the same.

So far, however, no definite place in the arts has been found for this absorbent fiber 40 outside of the use to which it has been put for many years, viz., as the principal ingredient of gun cotton and smokeless powder, for which purpose it has proved most successful. But with the ending of the war 45 this market has been absolutely closed and materials of this character have been without a market. It is the purpose of this invention to find a new and peace-time use for this material which should be manufactured 50 in a large way.

I have discovered that absorbent fibers of this character can be beaten or brushed out to substantially unify and straighten the fiber particles, and that after such treatment, the fiber can be placed in water and 55 flowed into a mold and compressed and dried

into a relatively dense and ponderous cubic body having a smooth surface, applied to many uses when there is desired a dense, solid, highly-absorbent body with a smooth 60 surface, such, for instance, as a blotter block as distinguished from an ordinary sheet of blotting paper.

The steps of my invention, therefore, consist in first beating or brushing out absorbent 65 cotton-seed hull fibers or linters; second, mixing the fibers with water; third, flowing the mass into a mold having perforate and imperforate surfaces; fourth, compressing while wet into a solid block; and fifth, 70 drying.

The resultant product is a unitary block, or solid body, the fibers being compactly matted, the respective surfaces of the cube being smooth on the top and bottom. Pref- 75 erably, the brushing or beating of the chemically prepared fibers is carried to such a point that the compressed and dried block, will be so hard and integral that its surfaces can be touched to a grinding disk, for shap- 80 ing, smoothing, fitting or finishing the block or its surfaces, and so contouring or surface-finishing the block as to adapt it to a particular selected usage.

A mold, such as is illustrated in the accom- 85 panying drawing, forming a part of this specification, is employed.

Figure 1 is a view of the mold.

Fig. 2 is a perspective view of the product.

It has the slotted or perforated sides 1, 90 the bottom 2, and the follower or plunger 3. being smooth and imperforate. The fibers are placed in a considerable volume of water and flowed into the mold. The water quickly and freely escapes from the fiber 95 through the perforate mold sections and the plunger is operated as soon as a mold is filled. The fiber is pressed into a condensed body or brick and dried, forming a heavy solid, absorbent fiber block or pad, the 100 smooth surfaces being on the top and bottom. The fibers are so intermatted that the resultant block constitutes a permanent, unitary structure, durable and integral.

A number of molds of this character can 105 readily be coördinated into a press for a continuous and large scale production.

It will readily be seen that simple, automatic and inexpensive machinery enables the production of compact, absorbent fiber blocks, 110 at a very low cost, because of the novel, simple and effective treatment steps, more par-

ticularly marked and important in comparison to the elaborate and costly machinery and processes employed when stocks of this character are made into paper.

5 It is essential to the purposes of my invention that the absorbent cotton fibers be relatively uniform and straight, in order to make a smooth surface.

It is also necessary that the fibers to be 10 treated shall be highly absorbent, for the compression of the saturated mass and the free flow of water therefrom under compression make possible that matting and inter-webbed condition which they assume under 15 the influence of the compression and rapid draining, and retain when dried. That is to say, a given fiber mass is mechanically suspended in a much greater volume of water, and at the same time, these fibers being so 20 highly and quickly absorbent, take up water to the point of saturation. When compressed, the water flows quickly and freely from the suspended fiber and also the absorbed water is quickly given up by the 25 fibers, leaving the fibers behind, and causing the individual fibers to inter-web as the water of suspension and absorption is forced out of the mass.

This fiber by-product is produced on a 30 large scale and has been practically valueless recently. It is therefore absolutely essential to find some very inexpensive method of converting this material into a stable commercial article, and this conjoint objective of a 35 cheap method of production and the formation of a very useful and marketable product, constitute the gist of this invention.

It is unnecessary to show a machine for 40 operating the plunger and mold indicated, or a series of them. At the end of the plunger stroke the mold should be raised to strip the finished block, and they can be

made in continuous operations on a large scale.

Having described my invention, I claim: 45

1. The art of forming absorbent cotton fibers into solid bodies, which consists in first beating and brushing out the fibers, second, mixing the fibers with water, and flowing into a compressing mold having perforate 50 and imperforate sections, third, pressing the mass while wet into a condensed block and lastly, substantially drying out the water.

2. The art of forming absorbent cotton fibers into compact, solid bodies, which consists in first unifying and straightening the fibers, second, mixing with water, third, compressing and intermatting the saturated fiber mass and imparting a smooth surface thereto, and lastly, in drying the condensed 60 block into a permanent, compact, solid body, having a property of hardness and integrality enabling a machine surfacing or contouring.

3. A highly absorbent cotton fiber block 65 comprising a dense, relatively ponderable solid body, the fibers of which are compacted and intermatted into a definite and substantially permanent structure.

4. A highly absorbent cotton fiber block 70 comprising a dense, relatively ponderable solid body, the fibers of which are compacted and intermatted into a definite and substantially permanent structure, having one of its surfaces substantially and relatively 75 smooth and uniform.

In witness whereof, I hereunto subscribe my name, as attested by the two subscribing witnesses.

WILLIAM C. JOHNSON.

Witnesses:

D. M. ARMSTRONG,  
W. B. LEWIS.